# EUROPEAN PATENT SPECIFICATION

(11) **EP 3 636 832 B1**
(45) Date of publication and mention of the grant of the patent: **06.12.2023**
(21) Application number: 18199295.9
(22) Date of filing: 09.10.2018
(51) Int. Cl.: D21H 27/00, D21H 17/34, D21H 19/20, D21H 19/56, D21H 19/82

(54) **A METHOD FOR MANUFACTURING A PAPER SUBSTRATE SUITABLE FOR A RELEASE LINER WITH HIGH CONTENT OF FUNCTIONAL VINYL GROUPS, AND PRODUCTS AND USES THEREOF**
VERFAHREN ZUR HERSTELLUNG EINES PAPIERSUBSTRATS, DAS FÜR EINE TRENNSCHICHT MIT HOHEM GEHALT AN FUNKTIONELLEN VINYLGRUPPEN GEEIGNET IST, SOWIE PRODUKTE UND VERWENDUNGEN DAVON
PROCÉDÉ DE FABRICATION D'UN SUBSTRAT DE PAPIER APPROPRIÉ POUR UNE DOUBLURE DÉTACHABLE À TENEUR ÉLEVÉE EN GROUPES VINYLIQUES FONCTIONNELS ET PRODUITS ET UTILISATIONS ASSOCIÉS

(43) Date of publication of application: 15.04.2020
(73) Proprietor: UPM-Kymmene Corporation, 00100 Helsinki (FI)
(72) Inventor: Kosonen, Harri, 53300 Lappeenranta (FI); Rissanen, Mikko, 02750 Espoo (FI); Littunen, Kuisma, 53100 Lappeenranta (FI); Rautalahti, Jaakko, 37630 Valkeakoski (FI); Antila, Janne, 13100 Hämeenlinna (FI)
(74) Representative: Berggren Oy

(56) References cited:
- EP-A1- 3 009 483
- US-A- 3 457 250
- US-A1- 2013 040 134
- US-A1- 2017 190 799

## Description

### Technical field

The invention relates to a paper substrate that is suitable for binding silicone in a catalytic hydrosilation reaction containing a high vinyl content polymer. The invention further relates to a method for manufacturing such paper substrate. The invention further relates to use of high-vinyl content polybutadiene in a method for manufacturing a paper substrate containing a high vinyl content polymer.

### Background

A release liner refers to a product comprising a paper substrate and a release layer (i.e. a cured release coating), such as a silicone-based release layer, applied on at least one side of the paper substrate. Release layers have a dehesive surface facing away from the paper substrate, the surface energy level typically being in the range of 21 to 25 dynes/cm. The dehesive surface of the release layer may be used to protect adhesive material in contact with the dehesive surface.

Papers used as paper substrates for siliconizing, such as glassine or supercalendered kraft paper, are typically manufactured from bleached chemical pulp, such as bleached Kraft pulp, with an aim to provide dimensionally stable and dense paper surface able to reduce the surface penetration of a release coating, when the release coating is applied on the paper surface. The surface penetration of the release coating can be further reduced by applying a coating (i.e. a primer layer) on the paper surface and/or calendaring the paper prior to applying the release layer. A primer layer typically applied on the paper surface is a surface coating. A conventional surface coating, also referred to as a "surface size", may improve the surface smoothness and reduce the porosity of the paper surface and thus act as a barrier between the release layer and the paper surface.

Release coatings based on silicone polymers are typically easy to apply and well-flowing. Uncured silicone polymers may penetrate easily into the pores of a paper, unless sufficient hydrophobicity is present at the paper surface. The curing of a silicone refers to a thermally induced cross-linking reaction of the silicone polymer once applied onto the substrate surface, which results into a cross-linked surface coating attached to the substrate surface. Release coatings have previously been cured by radiation, wherein the coating contains either an initiator in the formulation, such as a photo initiator sensitive to ultra violet light, or the curing relies on high-energy radiation, such as an electron beam, producing sufficient amounts of energy to start the cross-linking reaction. The radiation cured layer functioned by either breaking chemical bonds and/or generating ions, which resulted into a cured silicone polymer based release layer, without the use of additional heat.

Thermally curable release coatings refer to specific type of release coatings, which are distinguished from radiation curable systems. Low temperature curable silicone polymer or "LTC" silicone polymer, refers to an addition-curable polymer comprising silicone base polymer with functional vinyl groups and a cross-linker compound with silane hydride groups, which components are configured to cross-link in a catalytic hydrosilation reaction at a low temperature. In the presence of precious metal catalysts such as platinum or rhodium complexes, a silane hydride group undergoes an addition reaction with a vinyl group. The addition reaction is typically catalysed by a platinum catalyst. Platinum-catalyzed addition reactions are fast, and the curing speed of the reaction can be controlled via the curing temperature. A low temperature in this context refers to a catalytic hydrosilation reaction temperature of less than 120°C, preferably in the range of 55 to 110°C, wherein the silane hydride groups and the functional vinyl groups form covalently cross-linked structures within the release coating, thereby forming the cured release layer. Novel fast-curing silicone polymers are often further designed to function with low amounts of platinum catalyst.

A problem with respect to the fast-curing silicone polymers is the relatively low anchorage of the release coating applied on the paper substrate. Further, due to the high volumes of release liner material produced, there is a constant aim to reduce the amounts of platinum catalyst from the current level in the range of 50 to 35 ppm to a lower level, such as to a level of 30 ppm or below. Due to the wide use of fast-curing silicone polymers in release liners, there is a constant need to save costs by using less platinum. Platinum is a very expensive catalyst material. In addition, the amount of other reagents, such as silicone used for a release coating, is a cost factor to be minimized. A further challenge is the curing temperature, which refers to the minimum temperature wherein the silicone polymers begins to cross-link, such that a fixed layer structure with dehesive properties is obtained. The curing temperature should be maintained relatively low in order to save production costs due to heating. However, a very low curing temperature, e.g. below 45°C, may be problematic as the silicone polymers may then begin to cross-link prematurely, for example before it has been applied on the paper substrate surface. The importance of such parameters is emphasized when the machine speed is increased.

Thus far, the anchorage of fast-curing silicone polymers on the paper substrate has been improved by using a primer layer containing chemically post-treated polymer, such as water soluble polyvinyl alcohol, which has been modified to contain functional vinylic groups. In the chemical post-treatment of polyvinyl alcohol, the reaction typically takes place through the highly reactive hydroxyl group. A polymer containing hydroxyl groups is most often reacted with a compound that contains a carbonyl group. Carbonyl groups may be oxidized, and may undergo addition reactions under basic or neutral conditions. Hence, the modification of the polymer is performed by means of carbonyl group reactions with one or more hydroxyl groups of the polymer, thereby providing water soluble polymer modified to contain functional vinylic groups. Examples of carbonyl compounds are aldehydes, carboxylic acids, esters, anhydrides and acid halides. Examples of chemical post-treatment of polyvinyl alcohol by carbonyl group reactions are disclosed in publications WO 2009/147283 and WO 2011/104427, which disclose methods for grafting PVA polymer with organic molecule to provide the PVA polymer with vinylic functions.

A disadvantage related to chemical post-treatment of polyvinyl alcohol is, however, that when the amount of the carbonyl compound further containing a vinyl group in such a post-treatment reaction is increased, the solution quickly becomes highly viscose and increasingly less water-soluble. Hence, the solubility of the compounds significantly limits the amount of vinylic side groups that can be grafted into the PVA polymer. Attempts to increase the aldehyde content in the reaction solution dramatically increase the viscosity of the reaction solution such that the reactants will prematurely precipitate out of the solution. For example, when grafting polyvinyl alcohol, having a hydrolysis degree of 98 - 99 % and degree of polymerization of 1400, with undecylenic aldehyde (an aldehyde comprising 11 carbon atoms), the polymer typically becomes significantly less water-soluble already when undecylenic aldehyde is added to the reaction mixture more than 2% by weight, when expressed as grams of aldehyde compound per 100 grams of polyvinyl alcohol. The formed reaction product thus becomes highly viscose and very difficult to apply on a substrate surface as a coating. Hence the amount of vinylic side chains in a modified PVA polymer is maintained relatively low, which typically is necessitated by current high-speed release liner applications.

Due to the very limited amount of functional vinylic groups which can easily be grafted into a PVA polymer, previous solutions have not been able to provide a substrate without drawbacks in high-speed labelling applications. The higher the velocity in a labelling process is, the smaller is the acceptable amount of release liner silicone anchorage level defects.

### Summary

A silicone-based release layer comprises a base polymer containing functional vinyl groups (-CH=CH₂) and a cross-linker compound containing silane hydride (Si-H) groups. Novel fast-curing silicones can have a more branched molecular structure than those of the previous generation. The branched molecular structure enables faster reaction kinetics when cross-linking the functional vinyl groups (-CH=CH₂) and the cross-linker compound containing functional groups with silane hydride (Si-H) bonds. Novel fast-curing silicones therefore require less time for the addition curing reaction to take place.

A selectively addition-polymerized diene may be used to provide an oleophilic primer layer, which contains a polymer having high amounts of functional vinyl groups without styrene groups. The anchorage of a release layer to a paper substrate may thus be improved by providing a paper substrate having a primer layer surface containing a high amount of functional vinyl groups throughout the primer layer surface plane. A primer layer containing a high-vinyl content polymer provides an unprecedented means of improving the anchorage characteristics of a silicone-based release layer. In addition to fast curing silicone polymers which have been specifically referred to, the covalent attachment of other silicone polymers based on addition-curable cross-linker compound containing silane hydride bonds may also be improved.

A method for manufacturing polymer having high vinyl group content without a significant amount of hydroxyl groups may comprise selective polymerization of diene monomers. In particular, a method for manufacturing polymer having high vinyl group content may comprise reacting diene monomers having two or more vinylic groups in the presence of a catalyst selective for addition reaction. The percentage of the polymer repeat units containing a vinyl group may be adjusted by selecting the polymerization conditions and a suitable catalyst. A suitable catalyst is, for example, butyl lithium. The 1,3-butadiene monomer is highly selective for 1,2-addition reaction in the presence of butyl lithium, thereby producing high vinyl content polybutadiene that does not contain a significant amount of hydroxyl groups. High vinyl content polybutadiene may have a vinyl group content of up to 18,5 mmol/g, wherein the vinyl groups content represents the molality of the functional groups in the formed polymer.

The high amount of functional vinyl groups on a selectively addition-polymerized diene provides a composition which may be coated on a cellulose fiber-based paper, thereby providing a substrate improved anchorage properties toward silane hydride groups. A further advantage of such an oleophilic primer layer is the hydrophobicity of the surface. A hydrophobic primer layer may be used to resist the penetration of various substances, such as a water-based adhesive material, which may become into contact with the hydrophobic polymer coating. A hydrophobic polymer also evens out the characteristics of the whole surface, despite the existence of possible defects, such as holes, which may sometimes be present in the cellulose fiber-based paper.

Hydrophobic polymer coating, as such, has a poor adhesion to silicone. The silicone adhesion towards a hydrophobic polymer coating is furthermore inversely related to the coating speed. When the coating and curing is performed at higher speed, there is less adhesion of the silicone towards the hydrophobic polymer coating. When the cellulose fiber-based paper is, however, coated with a primer layer which contains a non-polar polymer having high vinyl group content without a significant amount of hydroxyl group, the polymer has a tendency to be hydrophobic and avoids the hydrophilic surface of the cellulose fibre-based paper. While a hydrophobic polymer coating, as such, has a poor adhesion to silicone, the catalytic hydrosilation reaction enables chemical bonding of the silicone with the functional vinylic group present in the polymer. An advantage of the hydrophobic surface on the cellulose fiber-based paper is that less adhesive may penetrate through a release layer into the cellulose fibre-based paper beneath, when the paper substrate is used as release liner paper substrate. Thus, also the minimum amount of force required to detach a label or excess matrix material is reduced. A further effect of the hydrophobic surface on the cellulose fiber-based paper is that this enables the thickness of the release layer to be reduced, since the minimum amount of force required to detach a label from the release liner is dependent of the thickness of the release layer. The hydrophobic surface therefore facilitates the reduction of the amounts of silicone and platinum required for providing a release layer. A thinner release layer further enables a lower high-speed release value. Without a significant amount of hydroxyl groups in the polymer the vinyl groups thereby have a tendency to orientate away from a hydrophilic surface, such as cellulose fiber-based paper, when coated on such a surface. A particular advantage of a primer layer that contains functional vinylic groups in an amount of equal to or higher than 0.3 mmol/g, preferably an amount of equal to or higher than 0.5 mmol/g in the formed polymer is that the high amount of functional vinyl groups enables the use of very fast curing silicone compounds in the release coating. When the polymer contains functional vinyl groups in an amount of equal to or higher than 0.5 millimoles per gram (mmol/g) of the polymer, this enables forming a tight, closed paper substrate with oleophilic properties on the surface. The cellulose fiber-based paper may be e.g. a coated paper having a grammage equal to or more than 38 g/m², for example in the range of 38 to 160 g/m². The formed paper substrate may therefore be arranged to have a tight, closed surface with oleophilic properties resembling those of a synthetic paper substrate surface. A synthetic material, such as polypropylene, conventionally tends to have a low surface energy level, and reduced anchorage of silicone to the substrate surface. However, as a significantly higher amount of vinyl groups compared to levels cited in the prior art can be provided on the paper substrate surface, this improves the anchorage of the silicone polymers cured via the polyaddition reaction.

While emulsions of styrene-butadiene copolymer (SBR) have been extensively used in coated papers due to low manufacturing cost, they in general are unsuitable for release liner primer layer applications. Styrene-butadiene copolymers for paper coatings, also denoted as SBR or SB-latex, are typically manufactured in the presence of emulsifying agents, such as surfactants like various soaps. The emulsifying agents are used to control the molecular weight and hence the viscosity of the formed copolymer product, but do not stay attached in the formation of copolymer and instead easily separate and float to the surface during manufacturing of the coating.

The polymerized diene comprising functional vinyl groups may further be arranged to contain unsaturated dicarboxylic acid or an anhydride or monoester thereof, such as maleic acid or maleic anhydride. Preferably, the polymeric primer layer having high amounts of functional vinyl groups, which is on top of the cellulose fiber-based paper, is without styrene groups. Thereby, a paper substrate having a surface without styrene groups may be obtained. The lack of styrene groups in the polymeric primer layer is related to the theoretical amount of functional vinyl groups obtainable on a polymer formed of monomers. Advantageously, the amount of functional vinyl groups in the polymer formed of monomers is maximized, which improves the hydrophobic properties of the polymer, as is the case with polybutadiene obtainable from 1,3-butadiene monomers by 1,2-addition polymerization. A further introduction of polar groups to the polymeric structure, such as the covalent grafting of unsaturated dicarboxylic acid, anhydride or monoester thereof, however, will consume said functional vinyl groups of the polymer. Polar groups which are covalently grafted to the vinylic groups of polymer structure therefore supercede part of the functional vinyl groups of the polymer. The amount of polar groups which have been covalently grafted to the polymer structure, however, may be used to control the hydrophobicity of the polymer, thereby selecting how the polymer behaves in water. A balance between the hydrophobic and hydrophilic properties of the polymer may be used to reduce problems commonly associated to emulsifying agents, which tend to separate easily and float to the surface. Such polar groups in the polymer composition may thus be arranged to modify the degree of hydrophobicity of the polymer composition. In particular, a polymerized diene may be arranged to contain hydrophilic groups to improve the water-solubility of the polymer composition, thereby facilitating the application of the polymer to a cellulose fiber-based paper layer. Namely, depending on the polymerization degree and the amount of hydrophilic groups in addition to the functional vinyl groups, the polymer composition may be water soluble or it may be applied as an water-based emulsion or water-based dispersion. Advantageously, the amount of unsaturated dicarboxylic acid or an anhydride or monoester thereof may be equal to or higher than 3 mol-% of the polymer. It is contemplated, that an amount of unsaturated dicarboxylic acid or an anhydride or monoester thereof in the range of 3 to 6 mol-% provides conditions suitable for a water-based emulsion. A water soluble polymer composition may be obtained, when the amount of unsaturated dicarboxylic acid or an anhydride or monoester thereof is equal to or higher than 20 mol-% and the solution has an alkaline pH, preferably a pH value above 8. Sodium salts may be used to improve solubility and stability of the polymer composition. A method for manufacturing polymer having high vinyl group content may thus further comprise grafting unsaturated dicarboxylic acid or an anhydride or monoester thereof, such as maleic acid or maleic anhydride, into the polymer having high vinyl group content, thereby modifying the hydrophobicity of the polymer.

There is provided a paper substrate that is suitable for binding silicone in a catalytic hydrosilation reaction, the paper substrate comprising
- a cellulose fiber-based paper and
- a polymeric primer layer,
wherein the polymeric primer layer comprises a polymer that contains functional vinyl groups in an amount of equal to or higher than 0.5 millimoles per gram (mmol/g) of the polymer, such that the surface of the primer layer is hydrophobic. Functional vinyl groups present on the surface of the primer layer are capable to form covalent bonds with a silicone-based release layer which may be applied on top of the hydrophobic primer layer.

There is provided a method for manufacturing a paper substrate that is suitable for binding silicone in a catalytic hydrosilation reaction, the method comprising
- providing a cellulose fiber-based paper and
- coating a polymeric primer on top of the cellulose fiber-based paper layer, thereby forming the paper substrate having a polymeric primer layer,
wherein the polymeric primer layer comprises a polymer that contains functional vinyl groups in an amount of equal to or higher than 0.5 millimoles per gram (mmol/g) of the polymer, such that the surface of the primer layer (PRIM1) is hydrophobic and the functional vinyl groups are capable to form covalent bonds with a silicone-based release layer (SIL1) applicable on top of the paper substrate (SUBST1).

Advantageously, the polymeric primer layer is made of or contains a polymerized diene compound comprising functional vinyl functional groups, such as high-vinyl content polybutadiene obtainable from 1,2-addition polymerization reaction of 1,3-butadiene.

Such a paper substrate could be used in a method for manufacturing a release liner, the method comprising
- providing a cellulose fiber-based paper and
- coating a polymeric primer that contains functional vinyl groups in an amount of equal to or higher than 0.5 millimoles per gram (mmol/g) of the polymer on top of the cellulose fiber-based paper, thereby forming the paper substrate having a hydrophobic surface layer comprising functional vinyl groups
- coating the hydrophobic surface layer with a silicone-based release layer comprising silane hydride groups, and
- curing the silicone-based release layer by means of a polyaddition reaction, thereby anchoring silicone-based release layer comprising silane hydride groups to the hydrophobic surface layer comprising functional vinyl groups, thereby forming the release liner.

Thus, in addition, there is also provided a release liner comprising
- a cellulose fiber-based paper,
- a hydrophobic surface layer that contains a polymerized diene, such as 1,2-addition polymerized polybutadiene, and
- a silicone-based release layer applied on top of the hydrophobic surface layer,
wherein the silicone-based release layer has been covalently anchored to the hydrophobic surface layer by means of a catalytic hydrosilation reaction.

High-vinyl content polybutadiene obtainable from 1,2-addition polymerization reaction may be used in a primer layer composition of a paper substrate suitable for binding silicone in a catalytic hydrosilation reaction. The polymerized diene compound may further contain unsaturated dicarboxylic acid or an anhydride or monoester thereof, such as maleic acid or maleic anhydride.

Advantageously, the polymeric primer layer contains a polymer comprising functional vinyl groups in an amount of equal to or higher than 2 millimoles per gram (mmol/g) of the polymer, preferably equal to or higher than 4 mmol/g, most preferably equal to or higher than 8 mmol/g. A higher amount of functional vinyl groups correlates directly with the hydrophobicity of the surface, thereby decreasing the surface energy, while still enabling silicone polymers to be cured via the polyaddition reaction. Experimental results have suggested that up to functional vinyl groups in an amount of 18.5 mmol/g of the polymer may be obtained on a primer layer applied on top of the cellulose fiber-based paper layer. Therefore, the amount of functional vinyl groups may be in the range of 0.5 to 18.5 mmol/g of the polymer, which amount represents the molality of the vinyl groups in the polymer.

The invention is described in the independent and dependent claims.

### Brief description of the drawings

- Figure 1: shows, by way of an example, a polyaddition reaction of a fast-curing silicone polymer in the presence of a platinum catalyst,
- Figure 2: shows, by way of an example, a facestock laminate attached on a release liner, the facestock laminate containing a face layer and an adhesive layer,
- Figure 3: shows, by way of an example, a primer layer containing a high vinyl content polymer applied on a cellulose fiber-based paper surface,
- Figure 4: shows, by way of an example, a method for manufacturing high vinyl content polymer from 1,3-butadiene monomers by 1,2-addition polymerization reaction in the presence of a selective catalyst,
- Figure 5: shows, by way of an example, a method for modifying the hydrophobicity of a polymer containing functional vinyl groups in high amounts by grafting the polymer with unsaturated dicarboxylic acid, anhydride or monoester thereof,
- Figure 6a: shows, by way of an example, a product containing a cellulose fiber-based paper surface coated with a primer layer containing a high vinyl content polymer, prior to arranging a silicone cross-linking reaction to take place between the high vinyl content polymer and a fast-curing silicone polymer applied on top of the primer layer containing functional vinyl group,
- Figure 6b: shows, by way of an example, a product containing a cellulose fiber-based paper surface coated with a primer layer containing a high vinyl content polymer, after a silicone cross-linking reaction has taken place to at least some extent between the high vinyl content polymer and a fast-curing silicone polymer applied on top of the primer layer containing functional vinyl group.

The drawings are schematic.

In the drawings, Sx and Sz denote orthogonal directions.

### Detailed description

Reference is made to Figures 1 and 2. Fast-curing silicone polymers are typically cured via a polyaddition reaction. A silicone-based release layer SIL1 (as denoted in Figure 2) may be formed in a polyaddition reaction of a silicone base polymer containing a functional vinyl group VIN1 and a cross-linker compound SH1 containing silane hydride bonds. The functional vinyl group VIN1 may be an end group or it may be positioned elsewhere in the silicone base polymer. A polyaddition reaction refers to a silicone cross-linking reaction, wherein a silicone base polymer containing a functional vinyl group VIN1 is arranged to form a covalent bond with a cross-linker compound SH1 in the presence of a catalyst compound. The catalyst compound is typically a metal catalyst, such as platinum catalyst, abbreviated as Pt. Fast-curing silicone polymers typically cross-link already at a temperature equal to or less than 100°C, such as in the range of 60 to 100°C. The activation temperature range and reaction kinetics may be adjusted by selecting the chemical composition of the silicone base polymer containing a functional vinyl group VIN1 and the chemical composition of the cross-linker compound SH1. Compositions having a cross-linking temperature close to room temperature of 25°C are not preferred, since this would increase the risk of premature silicone cross-linking reaction, before the compounds have been applied on the substrate surface.

Reference is made to Figures 2 and 3. A release liner REL1 may comprise a cellulose fiber-based paper PAP1 which may be cellulose fiber-based, a release layer SIL1 formed of a silicone resin, and an oleophilic primer layer PRIM1 between the cellulose fiber-based paper PAP1 and the release layer SIL1. A release liner REL1 may be used as backing material for a facestock laminate FILM1. A facestock laminate FILM1 is used for manufacturing adhesive labels. In such manufacturing, some of the facestock laminate FILM1 may be made e.g. by cutting discrete labels LAB1 out of the facestock laminate FILM1. Adhesive labels LAB1 may be, for example, self-adhesive labels or pressure sensitive labels formed of the facestock laminate FILM1. The release liner REL1 is provided with a dehesive surface in order to facilitate the separation of the facestock laminate FILM1 containing an adhesive layer ADH1 from the release liner REL1.

The paper substrate SUBST1 for a release liner REL1 denotes a combination of at least a cellulose fiber-based paper PAP1 and a primer layer PRIM1 as applied on at least one side of the cellulose fiber-based paper PAP1. The primer layer PRIM1 is typically applied on the side or sides intended to be coated with the silicone-based release layer SIL1. Advantageously, the primer layer PRIM1 is an oleophilic primer layer containing a polymerized diene PBUT1 having vinylic functions, said polymerized diene PBUT1 being present in the composition of the oleophilic primer layer PRIM1. When forming a release liner REL1, the primer layer PRIM1 is formed between the cellulose fiber-based paper PAP1 and the silicone-based release layer SIL1.

A method for manufacturing a release liner REL 1 may comprise providing a cellulose fiber-based paper PAP1. Examples of commercial products typically used as a release liner paper substrate SUBST1 are coated papers, vegetable parchment, glassine and greaseproof paper. Typical examples of coated papers are Super Calandered Kraft paper (SCK) and glassine. Glassine in general refers to paper made of chemical pulp, typically having a coat weight (grammage) in the range of 50 to 150 g/m². Glassine paper has a good transparency level; for example a 60 g/m² glassine paper typically has a transparency level of at least 45, when measured with visible light (ISO 2469:1994). Other examples of coated papers are Clay Coated Kraft paper (CCK), Machine Finished Kraft paper (MFK) and Machine Glazed paper (MG). Coated papers may have a grammage equal to or more than 38 g/m², such as in the range of 38 to 160 g/m².

A method for manufacturing a release liner REL1 may further comprise applying a primer layer PRIM1 on a cellulose fiber-based paper PAP1 surface. The primer layer PRIM1 may contain high vinyl content polymer PBUT1, such as a polymerized diene comprising functional vinyl groups VIN1, which is applied as a coating on top of the cellulose fiber-based paper PAP1, thereby forming a paper substrate SUBST1. A paper manufacturer typically provides the cellulose fiber-based paper PAP1 as a paper substrate SUBST1 comprising the primer layer PRIM1.

The primer layer PRIM1 surface may be arranged to have hydrophobicity. When the primer layer PRIM1 is arranged to contain a polymer comprising a catenated carbon structure, such as a linear chain of carbons without hydroxyl groups, the non-polar nature of the polymer is increased. Such polymer, when applied on a primer layer surface, therefore provides hydrophobicity and may thus be oleophilic. A hydrophobic primer layer PRIM1 surface may improve the orientation of functional vinyl groups VIN1 towards the surface of the primer layer PRIM1, thereby promoting the formation of covalent bonds with a silicone-based release layer SIL1, after a release coating has been applied on top of the hydrophobic primer layer PRIM1. A paper substrate SUBST1 may thus be arranged to have an oleophilic primer layer PRIM1 applied on top of a cellulose fiber-based paper PAP1 and covalent connections will be formed during the cross-linking of silicone, wherein the silane hydride groups of the cross-linker react with the vinyl groups VIN1 of the high vinyl content polymer PBUT1.

A method for manufacturing a release liner REL1 may further comprise coating the oleophilic primer layer PRIM1 with a silicone-based release layer SIL1. The silicone-based release layer SIL1 may comprise a fast-curing silicone polymer comprising cross-linker compound with silane hydride groups. The silicone-based release layer SIL1 may be cured by a polyaddition reaction in the presence of a catalyst, thereby anchoring the polymerized diene of the oleophilic primer layer to the silicone-based release layer SIL1, thereby forming the release liner REL1. The hydrophobicity of the primer layer PRIM1 improves the spreading of the silicone polymer applied on the paper substrate SUBST1, thereby enabling reducing the amount of silicone polymer needed to form a silicone-based release layer SIL1. The silicone-based release layer SIL1 may be applied later than during or immediately after manufacturing the paper substrate SUBST1, for example during manufacturing of the face stock FILM1. Alternatively, the silicone-based release layer SIL1 may be applied on the paper substrate SUBST1 during or immediately after manufacturing the paper substrate SUBST1, such as in the same production process and/or production line. An additional advantage of the hydrophobicity is, that a thinner release layer SIL1 may be provided, thereby reducing the amount of silicone polymer needed to form the silicone-based release layer SIL1. This subsequently will reduce the amount of platinum catalyst needed. The silicone-based release layer may thereby remain thin, such as less than 1 micrometer in thickness. A hydrophobic (i.e. oleophilic) paper substrate surface therefore facilitates the even spreading of the uncured silicone polymer applied on the surface. When the release liner paper substrate contains a polymer comprising functional vinyl groups in an amount of equal to or higher than 0.5 millimoles per gram of the polymer, the release layer SIL1 is more firmly bonded to the paper substrate. A hydrophobic primer layer may be used to resist the penetration of water-based or hot-melt adhesive material, which may be used in the manufacturing of a face stock FILM1 and may thus become into contact with the paper substrate SUBST1 surface. A hydrophobic polymer also evens out the characteristics, for example release characteristics, of the whole surface, despite the existence of possible defects, such as holes, which may sometimes be present in the cellulose fiber-based paper.

A removable facestock laminate FILM1 may be attached on a release liner REL1. The facestock laminate FILM1 may contain a face layer FACE1 and an adhesive layer ADH1 for attaching the facestock laminate FILM1 onto the release liner REL1 surface. The facestock laminate FILM1 may be used, for example to manufacture a label stock. Herein, a release liner REL1 carrying a plurality of adhesive labels is referred to as a label stock. A label stock is typically wound on a roll and used in a labelling process during which use the label stock is unwound as labels are needed.

Figure 3 illustrates a primer layer PRIM1 containing a high vinyl content polymer PBUT1 applied on a cellulose fiber-based paper PAP1 surface SURF1. A high vinyl content polymer PBUT1 refers to a polymer comprising functional vinyl groups VIN1 in an amount of equal to or higher than 0.5 millimoles per gram (mmol/g) of the polymer. Advantageously, the primer layer contains a polymer comprising functional vinyl groups in an amount of equal to or higher than 1 millimoles per gram (mmol/g) of the polymer, preferably equal to or higher than 2 mmol/g, most preferably equal to or higher than 4 mmol/g, such as equal to or higher than 8 mmol/g. The amount of functional vinyl groups may be, for example, in the range of 0.5 to 18.5 mmol/g of the polymer. A primer layer PRIM1 containing high vinyl content polymer PBUT1 is hydrophobic, as a large proportion of the functional vinyl groups VIN1 are present on the surface of the primer layer PRIM1. A higher amount of chains that end into functional vinyl groups correlates directly with the hydrophobicity of the surface, thereby decreasing the surface energy. Functional vinyl groups VIN1 present on the top surface of the primer layer PRIM1 (i.e. the surface facing away from cellulose fiber-based paper PAP1) are capable to form covalent bonds with a silicone-based release layer SIL1 which may be applied on top of the primer layer PRIM1. The primer layer PRIM1 may contain high vinyl content polymer PBUT1, such as polymerized diene.

Reference is made to Figure 4, illustrating an example of addition polymerization of 1,3-butadiene monomers.

A polymerized diene may be formed from diene monomers containing two or more functional vinyl groups VIN1 (-CH=CH₂) by means of a catalytic addition polymerization reaction. By using a selective catalyst, the polymerized diene may be arranged to contain a very high amount of functional vinyl groups VIN1.

In general, the chemical structure of a diene may be of the form

CH₂=CH-R-CH=CH₂

, wherein R refers to an optionally present carbon chain which may be linear, branched or cyclic, and may further contain heteroatoms.

A particular example of a suitable diene monomer is 1,3-butadiene, having the chemical structure of

CH₂=CH-CH=CH₂

1,3 -butadiene can be polymerized in three different ways, referred to as *cis-, trans-* and *vinyl*-additions, which result in different forms of polybutadiene. The cis and *trans* forms may be obtained in 1,4-addition reactions. High vinyl content polybutadiene may be obtained from 1,3 -butadiene by selective polymerization, when the polymerization is 1,2-addition reaction of 1,3-butadiene.

1,3-butadiene may be 1,2-addition polymerized in the presence of a selective catalyst, such as metallocene catalyst. A butyl lithium initiator as such may be used to provide 80-90 % of 1 ,4-addition product, as evidenced by Samotsvetov et al. (Butadiene polymerization in the presence of butyl lithium modified with sodium butylate, Polym Sci USSR 23 (1981) 100-107). However, when the reaction is done in the presence of 1,2-bis(piperidino)ethane, the selectivity towards 1,2-addition product may be up to 100%, as evidenced by Halasa, Lohr & Hall (Anionic polymerization to high vinyl polybutadiene, J Polym Sci Part A: Polym Chem 19 (1981) 1357-1360).

The letter n in Figure 4 refers to the amount of monomer units used to form a polymer. The reference sign CAT1, in turn, refers to the catalyst used for the polymerization reaction. The n may be, for example in the range of 10 to 10000, thereby providing a polybutadiene having a molecular weight in the range of 110 to 540000 g/mol.

Reference is made to Figures 5 and 6a and 6b. The oleophilic primer layer PRIM1 between the cellulose fiber-based paper PAP1 and the release layer SIL1 may further contain solubilizing agent between 3 mol-% and 20 mol-% of the polymer, such that the high vinyl content polymer PBUT1 comprising functional vinyl groups is water-dispersible or water-emulsifiable, when applied on top of the cellulose fiber-based paper PAP1. Further, the high vinyl content polymer PBUT1 may contain solubilizing agent in an amount equal to or higher than 20 mol-% of the polymer, such that the polymer comprising functional vinyl groups is water-soluble, when applied on top of the cellulose fiber-based paper PAP1. The solubilizing agent may be, for example, an unsaturated dicarboxylic acid or an anhydride or monoester thereof, such as maleic acid or maleic anhydride, which has been grafted into the high vinyl content polymer PBUT1 comprising the functional vinyl groups, as shown in Figure 5. Alternatively, an unsaturated carboxylic acid or an unsaturated acrylic containing a functional vinyl group may be used. The improved water-solubility of a polymer composition comprising the high vinyl content polymer PBUT1 facilitates the homogeneous application of the polymer composition on a cellulose fiber-based paper PAP1 surface. The silicone layer and excess cross-linker compound SH1 is thereby bonded covalently and more strongly to the substrate surface.

### Example 1 - preparation of high-vinyl content polybutadiene

In an experiment, 400 g (7.4 mol) of 1,3-butadiene was weighted and subsequently dissolved in 1600 g of cyclohexane under nitrogen atmosphere, such that a clear solution containing 1,3-butadiene monomers was obtained. The temperature of the solution containing the 1,3-butadiene monomers was then adjusted to 30°C, and an initiator system comprising 0.17 g (2.65 mmol) of butyl lithium and 5.2 g (26.5 mmol) of 1,2-bis(piperidino)ethane was added, thereby providing a reaction mixture and reaction conditions selective for 1,2-addition reaction of 1,3-butadiene. The reaction mixture was then agitated for 120 min with a mechanical stirrer, after which 2000 g of ethanol was added to stop the reaction and precipitate the polymer. The reaction product was purified by evaporating solvent and monomer residues at 50°C in vacuum. The purified polybutadiene had number average molecular weight of 150000 g/mol, analyzed by size exclusion chromatography (abbreviated as SEC), and included 99 mol-% of 1 ,2-addition product, when analyzed by nuclear magnetic resonance (abbreviated as NMR).

### Example 2 - experimental data of high-vinyl content polybutadiene

Table 1 (below) demonstrates a correlation between vinyl percentage, i.e. the percentage of the polymer repeat units containing a vinyl group, and the vinyl group content (mmol/g). As can be seen from the Table 1, when 1,3-butadiene is 1,2-addition polymerized in the presence of a selective catalyst, a very high vinyl content may be obtained. A higher amount of functional vinyl groups in polybutadiene has been observed to correlate with higher hydrophobicity on coated cellulose fiber-based papers, thereby indicating that higher amounts of functional vinyl groups on the surface decrease the surface energy. When the vinyl content is very high, such as higher than 60 percent of the amount of polymer repeat units, the reaction conditions may be selected to produce polybutadiene having lower molecular weight. A lower molecular weight of the polybutadiene may be advantageous for reducing the risk of premature cross-linking of the polybutadiene repeat units.

**Table 1. Comparison of vinyl group molality (mmol/g) between polymerized butadiene (polybutadiene) grades as a function of vinyl percent of polymer. The 'vinyl percent of polybutadiene' in this context refers to the percentage of the polymer repeat units containing a vinyl group. The 'vinyl content in this context refers to the classification of the polybutadiene with respect to the vinyl content. Normal (conventional) catalyst and reaction route typically results to a butadiene having vinyl groups in the range of 1 to 2 percent of the amount of polymer repeat units. Upon butyl lithium catalyst and 1,2-bis(piperidino)ethane initiator system, polybutadiene having increased amount of vinyl groups may be obtained.**

| **vinyl percentage of polybutadiene** | **vinyl group molality (mmol/g)** | **vinyl content** |
|---|---|---|
| 1 | 0.19 | normal |
| 2 | 0.37 | normal |
| 4 | 0.74 | increased |
| 6 | 1.11 | increased |
| 10 | 1.85 | increased |
| 20 | 3.70 | increased |
| 30 | 5.56 | high |
| 40 | 7.41 | high |
| 50 | 9.26 | high |
| 60 | 11.11 | high |
| 80 | 14.81 | high |
| 90 | 16.67 | high |

### Comparative example 3 - vinyl group content obtainable by post-grafting polyvinyl alcohol

A comparative experiment was performed to demonstrate the level of vinyl group contents achievable by grafting polyvinyl alcohol with an organic molecule containing a functional vinyl group in an acetalization reaction. When grafting polyvinyl alcohol having a hydrolysis degree of 98 - 99 % and degree of polymerization of 1400 with 10-undecenal (an aldehyde comprising 11 carbon atoms), the polymer became significantly less water-soluble already when 10-undecenal was added 3 wt.-%, when expressed as grams of aldehyde compound per 100 grams of polyvinyl alcohol. The formed reaction product further became highly viscose and such that application of the reaction product on a substrate surface as a coating was not feasible by conventional coating means. The results of the comparative experiment are presented in Table 2 (below).

**Table 2. Comparison of vinyl group contents in modified polyvinyl alcohol samples as a function of the aldehyde reactant content (10-undecenal, molecular weight of 168 g/mol). The 'degree of modification (wt-%)' refers to the mass ratio (in percentages) of the aldehyde reactant in grams that has been reacted per 100 grams of the polyvinyl alcohol. The 'coatability' refers to the coatability of the reaction product to a cellulose fibre-based paper, wherein the formed polymer product is either easy to coat (`1') such that reaction product viscosity is low enough to apply by conventional coating means, or the polymer is difficult to coat (`2') such that that reaction product forms a viscose gel which is not easy to apply by conventional coating means, or the polymer has lost its coatability (`3') to such a degree that the reaction product could no longer be applied as a coating.**

| degree of modification (wt-%) | vinyl group molality (mmol/g) | coatability |
|---|---|---|
| 0 | 0 | 1 |
| 1 | 0.06 | 1 |
| 2 | 0.12 | 2 |
| 3 | 0.17 | 3 |
| 3.5 | 0.20 | 3 |
| 4 | 0.23 | 3 |
| 5 | 0.28 | 3 |
| 10 | 0.55 | 3 |
| 15 | 0.79 | 3 |
| 20 | 1.01 | 3 |
| 25 | 1.21 | 3 |
| 30 | 1.41 | 3 |

### NMR method to evaluate the quantity of functional vinyl groups

Proton nuclear magnetic resonance (¹H-NMR) analysis may be used to identify chemical structures from the chemical shift values δ of individual hydrogen atoms. Samples for ¹H-NMR analysis may be prepared by dissolving PBD into a suitable solvent, such as deuterated chloroform.

Further, integration of the ¹H-NMR spectra may be used to estimate vinyl group content of PBD samples. This can be accomplished by comparing areas of the peaks representing the terminal vinyl protons in 1,2-addition product (6 = 4.8 ppm) and olefinic protons in 1,4-addition product (δ = 5.4 ppm). The molality (mmol/g) of vinyl groups in the product can be calculated according to equation 1. ${b}_{1,2} = \frac{{A}_{1,2}}{{A}_{1,2} + {A}_{1,4}} \times \frac{1000 \frac{mmol}{mol}}{{M}_{BD}}$ where b_{1,2} represents the molality (mmol/g) of vinyl groups, A_{1,2} and A_{1,4} represent the integrated areas of the peaks representing terminal vinyl protons and 1,4-olefinic protons, respectively, and M_{BD} represents the molecular weight of butadiene.

For example, when in a tested polybutadiene sample the integrated area of the NMR spectra of 1,4-olefinic protons is 36 and the integrated area of the NMR spectra of the terminal vinyl protons is 1, the tested polybutadiene sample having a molecular weight of 54.09 g/mol, the tested polybutadiene sample has a molality of 0.5 mmol/g of vinyl groups, as demonstrated below using Equation 1: ${b}_{1,2} = \frac{1}{1 + 36} \times \frac{1000 \frac{mmol}{mol}}{54.09 \frac{g}{mol}} = 0.5 mmol / g$

## Claims

1. A paper substrate (SUBST1) that is suitable for binding silicone in a catalytic hydrosilation reaction, the paper substrate (SUBST1) comprising
- a cellulose fiber-based paper (PAP1) and
- a polymeric primer layer (PRIM1),
wherein the polymeric primer layer (PRIM1) comprises a polymer that contains functional vinyl groups in an amount of equal to or higher than 0.5 millimoles per gram of the polymer, such that the surface of the polymeric primer layer (PRIM1) is hydrophobic, wherein the polymer that contains functional vinyl groups is high-vinyl content polybutadiene, which is an isomeric form of polybutadiene obtainable from 1,3-butadiene monomers by 1,2-addition polymerization.

2. A method for manufacturing a paper substrate (SUBST1) that is suitable for binding silicone in a catalytic hydrosilation reaction, the method comprising
- providing a cellulose fiber-based paper (PAP1) and
- coating a polymeric primer layer (PRIM1) on top of the cellulose fiber-based paper (PAP1), thereby forming the paper substrate (SUBST1), wherein the polymeric primer layer (PRIM1) comprises a polymer that contains functional vinyl groups in an amount of equal to or higher than 0.5 millimoles per gram of the polymer, such that the surface of the primer layer (PRIM1) is hydrophobic and the functional vinyl groups are capable to form covalent bonds with a silicone-based release layer (SIL1) applicable on top of the paper substrate (SUBST1), wherein the polymer that contains functional vinyl groups is high-vinyl content polybutadiene, which is an isomeric form of polybutadiene obtainable from 1,3-butadiene monomers by 1,2-addition polymerization.

3. The method according to claim 2, further comprising
- polymerizing diene monomers comprising functional vinyl groups in an addition polymerization reaction, thereby forming the polymer that contains functional vinyl groups.

4. The method according to claim 3, wherein
- the addition polymerization reaction is catalyzed by butyl lithium and, when necessary, in the presence of 1,2-bis(piperidino)ethane initiator system.

5. The method according to any of the claims 2 to 4, wherein the polymer that contains functional vinyl groups further contains solubilizing agent between 3 mol-% and 20 mol-% of the polymer, such that the polymer comprising functional vinyl groups is water-dispersible or water-emulsifiable, when applied on top of the cellulose fiber-based paper (PAP1).

6. The method according to any of the previous claims 2 to 4, wherein the polymer that contains functional vinyl groups further contains solubilizing agent in an amount equal to or higher than 20 mol-% of the polymer, such that the polymer comprising functional vinyl groups is water-soluble, when applied on top of the cellulose fiber-based paper (PAP1).

7. The method according to the previous claim 5 or 6, wherein the solubilizing agent is an unsaturated dicarboxylic acid or an anhydride or monoester thereof, such as maleic acid or maleic anhydride, which has been grafted into the polymer that contains functional vinyl groups.

8. The paper substrate (SUBST1) according to claim 1 or the method according to any of the claims 2 to 7, wherein the polymeric primer layer (PRIM1) comprises a polymer that contains functional vinyl groups in an amount of equal to or higher than 2 millimoles per gram of the polymer, preferably equal to or higher than 4 millimoles per gram of the polymer, most preferably equal to or higher than 8 millimoles per gram of the polymer.

9. The paper substrate (SUBST1) or the method according to any of the previous claims, wherein the cellulose fiber-based paper (PAP1) is coated paper having a grammage equal to or more than 38 g/m², for example in the range of 38 to 160 g/m².

10. The paper substrate (SUBST1) or the method according to any of the previous claims, wherein the polymeric primer layer (PRIM1) applied on top of the cellulose fiber-based paper (PAP1) is applied in an amount of 0.1 to 20 g/m², preferably in an amount of 1 to 5 g/m².

11. The paper substrate (SUBST1) or the method according to any of the previous claims, wherein the polymeric primer layer (PRIM1) applied on top of the cellulose fiber-based paper (PAP1) contains the polymer comprising functional vinyl groups equal to or more than 1 wt.%, such as in the range of 1 to 100 wt.% of the weight of the polymeric primer layer (PRIM1).

12. The paper substrate (SUBST1) or the method according to any of the previous claims, wherein the polymeric primer layer (PRIM1) applied on top of the cellulose fiber-based paper (PAP1) is without styrene groups.

13. Use of a high-vinyl content polybutadiene, which is an isomeric form of polybutadiene obtainable from 1,3-butadiene monomers by 1,2-addition polymerization, comprising functional vinyl groups in a primer layer composition of a paper substrate suitable for binding silicone in a catalytic hydrosilation reaction.

## Patentansprüche

1. Ein Papierträgermaterial (SUBST1), das zum Binden von Silikon in einer katalytischen Hydrosilylierungsreaktion geeignet ist, wobei das Papierträgermaterial (SUBST1) umfasst
- ein Papier auf Zellulosefaserbasis (PAP1) und
- eine Polymerprimerschicht (PRIM1),
wobei die Polymerprimerschicht (PRIM1) ein Polymer umfasst, das funktionelle Vinylgruppen in einer Menge von 0,5 Millimol oder mehr pro Gramm des Polymers enthält, so dass die Oberfläche der Polymerprimerschicht (PRIM1) hydrophob ist, wobei das Polymer, das funktionelle Vinylgruppen enthält, Polybutadien mit hohem Vinylgehalt ist, das eine isomere Form von Polybutadien ist, das aus 1,3-Butadienmonomeren durch 1,2-Additionspolymerisation erhältlich ist.

2. Ein Verfahren zur Herstellung eines Papierträgermaterials (SUBST1), das zum Binden von Silikon in einer katalytischen Hydrosilylierungsreaktion geeignet ist, wobei das Verfahren umfasst
- die Bereitstellung eines Papiers auf Zellulosefaserbasis (PAP1) und
- die Beschichtung einer Polymerprimerschicht (PRIM1) auf dem Papier auf Zellulosefaserbasis (PAP1), wodurch das Papierträgermaterial (SUBST1) gebildet wird, wobei die Polymerprimerschicht (PRIM1) ein Polymer umfasst, das funktionelle Vinylgruppen in einer Menge von 0,5 Millimol oder mehr pro Gramm des Polymers enthält, so dass die Oberfläche der Polymerprimerschicht (PRIM1) hydrophob ist und die funktionellen Vinylgruppen in der Lage sind, kovalente Bindungen mit einer Trennschicht (SIL1) auf Silikonbasis zu bilden, die auf das Papierträgermaterial (SUBST1) aufgebracht werden kann, wobei das Polymer, das funktionelle Vinylgruppen enthält, Polybutadien mit hohem Vinylgehalt ist, das eine isomere Form von Polybutadien ist, das aus 1,3-Butadien-Monomeren durch 1,2-Polyaddition erhalten werden kann.

3. Das Verfahren nach Anspruch 2, umfassend ferner
- die Polymerisierung von Dienmonomeren, die funktionelle Vinylgruppen enthalten, in einer Polyadditionsreaktion, wodurch das Polymer gebildet wird, das funktionelle Vinylgruppen enthält.

4. Das Verfahren nach Anspruch 3, wobei
- die Polyadditionsreaktion durch Butyllithium und, falls erforderlich, in Gegenwart eines 1,2-Bis(piperidino)ethan-Initiatorsystems katalysiert wird.

5. Das Verfahren nach einem der Ansprüche 2 bis 4, wobei das Polymer, das funktionelle Vinylgruppen enthält, ferner ein Lösungsvermittlungsmittel zwischen 3 Mol-% und 20 Mol-% des Polymers enthält, so dass das Polymer, das funktionelle Vinylgruppen umfasst, wasserdispergierbar oder wasseremulgierbar ist, wenn es auf das Papier auf Zellulosefaserbasis (PAP1) aufgetragen wird.

6. Das Verfahren nach einem der vorhergehenden Ansprüche 2 bis 4, wobei das Polymer, das funktionelle Vinylgruppen enthält, weiterhin ein Lösungsvermittlungsmittel in einer Menge von 20 Mol-% oder mehr des Polymers enthält, so dass das Polymer, das funktionelle Vinylgruppen umfasst, wasserlöslich ist, wenn es auf das Papier auf Zellulosefaserbasis (PAP1) aufgetragen wird.

7. Das Verfahren nach dem vorhergehenden Anspruch 5 bzw 6, wobei es sich bei dem Lösungsvermittler um eine ungesättigte Dicarbonsäure oder ein Anhydrid oder einen Monoester davon, wie Maleinsäure oder Maleinsäureanhydrid, handelt, die bzw. der auf das Polymer, das funktionelle Vinylgruppen enthält, aufgebracht worden ist.

8. Das Papierträgermaterial (SUBST1) nach Anspruch 1 oder das Verfahren nach einem der Ansprüche 2 bis 7, wobei die Polymerprimerschicht (PRIM1) ein Polymer umfasst, das funktionelle Vinylgruppen in einer Menge von 2 Millimol oder mehr pro Gramm des Polymers, vorzugsweise von 4 Millimol oder mehr pro Gramm des Polymers, am meisten bevorzugt von 8 Millimol oder mehr pro Gramm des Polymers enthält.

9. Das Papierträgermaterial (SUBST1) oder das Verfahren nach einem der vorhergehenden Ansprüche, wobei das Papier auf Zellulosefaserbasis (PAP1) ein beschichtetes Papier mit einem Flächengewicht von 38 g/m² oder mehr, beispielsweise im Bereich von 38 bis 160 g/m², ist.

10. Das Papierträgermaterial (SUBST1) oder das Verfahren nach einem der vorhergehenden Ansprüche, wobei die Polymerprimerschicht (PRIM1), die auf das Papier auf Zellulosefaserbasis (PAP1) aufgetragen wird, in einer Menge von 0,1 bis 20 g/m², vorzugsweise in einer Menge von 1 bis 5 g/m², aufgebracht wird.

11. Das Papierträgermaterial (SUBST1) oder das Verfahren nach einem der vorhergehenden Ansprüche, wobei die Polymerprimerschicht (PRIM1), die auf das Papier auf Zellulosefaserbasis (PAP1) aufgebracht wird, das Polymer enthält, das funktionelle Vinylgruppen in Höhe von 1 Gew.-% oder mehr, wie etwa in einem Bereich von 1 bis 100 Gew.-% des Gewichts der Polymerprimerschicht (PRIM1), umfasst.

12. Das Papierträgermaterial (SUBST1) oder das Verfahren nach einem der vorhergehenden Ansprüche, wobei die Polymerprimerschicht (PRIM1), die auf das Papier auf Zellulosefaserbasis (PAP1) aufgebracht wird, keine Styrolgruppen enthält.

13. Die Verwendung eines Polybutadiens mit hohem Vinylgehalt, bei dem es sich um eine isomere Form von Polybutadien handelt, das aus 1,3-Butadien-Monomeren durch 1,2-Polyaddition erhältlich ist, das funktionelle Vinylgruppen in einer Primerschichtzusammensetzung eines Papierträgermaterials enthält, das zur Bindung von Silikon in einer katalytischen Hydrosilylierungsreaktion geeignet ist.

## Revendications

1. Substrat en papier (SUBST1) approprié pour lier du silicone dans une réaction d'hydrosilation catalytique, le substrat en papier (SUBST1) comprenant
- un papier à base de fibres de cellulose (PAP1) et
- une couche primaire polymère (PRIM1),
dans lequel la couche primaire polymère (PRIM1) comprend un polymère qui contient des groupes vinyle fonctionnels en une quantité égale ou supérieure à 0,5 millimole par gramme du polymère, de sorte que la surface de la couche primaire polymère (PRIM1) est hydrophobe, dans lequel le polymère qui contient des groupes vinyle fonctionnels est un polybutadiène à haute teneur en vinyle, qui est une forme isomère de polybutadiène pouvant être obtenue à partir de monomères de buta-1,3-diène par polymérisation par addition 1,2.

2. Procédé de fabrication d'un substrat en papier (SUBST1) approprié pour lier du silicone dans une réaction d'hydrosilation catalytique, le procédé comprenant
- la fourniture d'un papier à base de fibres de cellulose (PAP1) et
- le couchage d'une couche primaire polymère (PRIM1) sur le papier à base de fibres de cellulose (PAP1), formant ainsi le substrat en papier (SUBST1), dans lequel la couche primaire polymère (PRIM1) comprend un polymère qui contient des groupes vinyle fonctionnels en une quantité égale ou supérieure à 0,5 millimole par gramme du polymère, de sorte que la surface de la couche primaire (PRIM1) est hydrophobe et les groupes vinyle fonctionnels peuvent former des liens covalents avec une couche de libération à base de silicone (SIL1) pouvant être appliquée sur le substrat en papier (SUBST1), dans lequel le polymère qui contient des groupes vinyle fonctionnels est un polybutadiène à haute teneur en vinyle, qui est une forme isomère de polybutadiène pouvant être obtenue à partir de monomères de buta-1,3-diène par polymérisation par addition 1,2.

3. Procédé selon la revendication 2, comprenant également
- la polymérisation de monomères diènes comprenant des groupes vinyle fonctionnels dans une réaction de polymérisation par addition, formant ainsi le polymère qui contient des groupes vinyle fonctionnels.

4. Procédé selon la revendication 3, dans lequel
- la réaction de polymérisation par addition est catalysée par le butyl lithium et, si nécessaire, en présence de système initiateur 1,2-bis(pipéridino)éthane.

5. Procédé selon l'une quelconque des revendications 2 à 4, dans lequel le polymère qui contient des groupes vinyle fonctionnels contient également un agent solubilisant entre 3% en moles et 20% en moles du polymère, de sorte que le polymère comprenant des groupes vinyles fonctionnels est dispersible dans l'eau ou émulsionnable à l'eau, lorsqu'il est appliqué sur le papier à base de fibres de cellulose (PAP1).

6. Procédé selon l'une quelconque des revendications précédentes 2 à 4, dans lequel le polymère qui contient des groupes vinyle fonctionnels contient également un agent solubilisant en une quantité égale ou supérieure à 20% en moles du polymère, de sorte que le polymère comprenant des groupes vinyle fonctionnels est soluble dans l'eau, lorsqu'il est appliqué sur le papier à base de fibres de cellulose (PAP1).

7. Procédé selon la revendication précédente 5 ou 6, dans lequel l'agent solubilisant est un acide dicarboxylique insaturé ou un anhydride ou monoester de celui-ci, tel que l'acide maléique ou l'anhydride maléique, qui a été greffé dans le polymère qui contient des groupes vinyle fonctionnels.

8. Substrat en papier (SUBST1) selon la revendication 1 ou procédé selon l'une quelconque des revendications 2 à 7, dans lequel la couche primaire polymère (PRIM1) comprend un polymère qui contient des groupes vinyle fonctionnels en une quantité égale ou supérieure à 2 millimoles par gramme du polymère, de préférence égale ou supérieure à 4 millimoles par gramme du polymère, de préférence égale ou supérieure à 8 millimoles par gramme du polymère.

9. Substrat en papier (SUBST1) ou procédé selon l'une quelconque des revendications précédentes, dans lequel le papier à base de fibres de cellulose (PAP1) est un papier couché ayant un grammage égal ou supérieur à 38 g/m², par exemple compris dans la plage de 38 à 160 g/m².

10. Substrat en papier (SUBST1) ou procédé selon l'une quelconque des revendications précédentes, dans lequel la couche primaire polymère (PRIM1) appliquée sur le papier à base de fibres de cellulose (PAP1) est appliquée en une quantité de 0,1 à 20 g/m², de préférence en une quantité de 1 à 5 g/m².

11. Substrat en papier (SUBST1) ou procédé selon l'une quelconque des revendications précédentes, dans lequel la couche primaire polymère (PRIM1) appliquée sur le papier à base de fibres de cellulose (PAP1) contient le polymère comprenant des groupes vinyle fonctionnels, égal ou supérieur à 1% en poids, par exemple dans la plage de 1 à 100% en poids du poids de la couche primaire polymère (PRIM1) .

12. Substrat en papier (SUBST1) ou procédé selon l'une quelconque des revendications précédentes, dans lequel la couche primaire polymère (PRIM1) appliquée sur le papier à base de fibres de cellulose (PAP1) est dépourvue de groupes styrène.

13. Utilisation d'un polybutadiène à haute teneur en vinyle, qui est une forme isomère de polybutadiène pouvant être obtenue à partir de monomères de buta-1,3-diène par polymérisation par addition 1,2, comprenant des groupes vinyle fonctionnels dans une composition de couche primaire d'un substrat en papier approprié pour lier du silicone dans une réaction d'hydrosilation catalytique.
